

Patented Mar. 20, 1928.

1,662,951

# UNITED STATES PATENT OFFICE.

ALFRED O. BRAGG, OF NIAGARA FALLS, NEW YORK, ASSIGNOR TO INTERNATIONAL BLEACHING CORPORATION, A CORPORATION OF DELAWARE.

## PROCESS OF BLEACHING ANIMAL AND VEGETABLE MATERIALS.

No Drawing.

Application filed September 5, 1925. Serial No. 54,818.

This invention relates to new and useful improvements in processes of bleaching animal and vegetable materials, but is designed more specially for use in a process 5 for bleaching ground wood pulp, and has for its principal objects:

First, to increase the efficiency and speed with which such bleaching is carried out, particularly with reference to ground wood 10 pulp.

Second, to effect a great increase in the degree of activity and effectiveness of the fundamental bleaching agents operative in the present bleaching processes, by a wholly 15 different treatment.

Third, to produce a bleached ground wood pulp of higher quality than is obtained by present methods.

Further objects, apparent to those skilled 20 in the art, will appear from the following description.

The process of the present invention is suitable for use in bleaching substances other than ground wood pulp capable of being 25 bleached by sulphurous acid such as, for example, palm leaf, straw, silk, cane, wool, etc.

In the following description and claims, the term "animal and vegetable materials" 30 will be understood to include such substances, the bleaching of ground wood pulp being the preferable application of the invention.

The existing methods of bleaching ground wood pulp are carried out by applying to the pulp, at densities from about 30% to 35 45% bone dry pulp, a solution of sodium or calcium bisulphite and, at times, concentrated sulphuric acid. The pulp, in laps, is allowed to remain in the air for one or two days or longer, for the bleaching to become 40 completed as far as possible, and the bleaching chemicals are applied to the pulp on the couch roll of the wet press, or similar machine.

The bleaching is presumably effected by 45 both sulphonation of the coloring matter of the pulp to form soluble, colorless, coloring-matter sulphonates, and also by reduction. The first reactions are made by the sulphurous acid itself and the second, by the nascent 50 hydrogen evolved from the sulphurous acid.

The bleaching of ground wood pulp at present is done both with, and without, the use of sulphuric acid to speed up the bleaching by rapid evolution of free sulphurous 55 acid from the bisulphite.

These methods have serious disadvantages, including irregularities in the application of the bisulphite solution, due to inherent short-comings in the equipment used, frequently resulting in streaked or incompletely 60 bleached pulp.

The space required for storing the pulp while bleaching moreover, is large, and costly, and interferes with other mill operations. The bleached pulp retains an odor 65 of sulphurous acid, due to chemical residues left in it. These residues cause trouble and expense in manufacturing paper from the pulp, such as decolorizing of aniline dyes, corrosion of equipment, acid in the paper, 70 etc.

The labor necessary for piling the pulp for the storage period during bleaching, and for unpiling it for use, is considerable. The permanence of the color obtained is not sufficiently great for many purposes, and the degree of "whiteness" obtainable is often 75 insufficient.

Usually, only new ground wood pulp, as it is being manufactured, can be bleached, as 80 the wet presses or equivalent equipment are ordinarily an integral part of the ground wood pulp manufacturing process. Because of this last condition, the existing methods do not permit of being efficiently used with 85 the other methods and equipment of the mill. Lastly, the bleaching is very slow.

A further object of the invention is to avoid the foregoing difficulties and disadvantages as well as to greatly increase the 90 efficiency, speed and quality of the bleaching.

I have discovered that, if ground wood pulp be circulated in water at densities of from 4% to 40% bone dry pulp and at temperatures of from 80° F. to 200° F., with a 95 mixture of a bisulphite or bisulphites, an acid other than sulphurous acid, and free sulphurous acid; and finally, if the pulp be washed with water until free of acid and other undesired materials, the foregoing objects are attained, and the pulp is bleached free from the above disadvantages and in the most facile, economical and satisfactory manner. It may be added that under ordinary conditions the temperature above referred to should not be over 165° F. because of the danger of darkening the pulp. There are conditions where greater temperatures would not darken the pulp, but they would not usually be met with in practice. 100 105 110

I have further discovered that if nascent hydrogen in larger amounts than is evolved from the amount of sulphurous acid used, be kept in contact with the pulp while it is being bleached as described above, the permanence and whiteness of the bleach is improved and the speed of the bleaching process is considerably increased.

It should be understood, however, that the practice of my process, without the nascent hydrogen as described, produces faster bleaching, and a better color and permanence to the bleach than present methods, due to the fact that both the sulphonation and reduction are greatly accelerated by the conditions of my process.

The details of carrying out my process admit of several variations, which will be apparent to those skilled in the art, without departure from the spirit of the invention, which resides in circulating the ground wood pulp with sulphurous acid, and then washing the pulp, so as to remove the acids and other undesirable material therefrom.

25 The following is given as an illustration of the method of the invention as applied to ground wood pulp.

Ground wood pulp and water are mixed in the proportions of about 7% bone dry pulp and about 93% water. To each 2,000 pounds of the bone dry pulp, there are added about 115 pounds of sodium bisulphite, 20 or 25 pounds of concentrated sulphuric acid (66 degrees Baumé) and 10 pounds of sodium hydrosulphite, as reducing material. These chemicals are preferably dissolved in water and then added to the pulp.

The mixture is then circulated for one or two hours within a temperature range of 40 from 80° F. to 200° F., but usually at a temperature of 130-150 degrees Fahrenheit. It is then washed with water until free from acids and other undesired materials, and the pulp is bleached, cleansed and ready for use.

45 My invention is not limited to any particular bleaching or washing equipment, as any apparatus of suitable construction and adapted to carrying out the process may be used. The invention is not limited moreover to any specific means for obtaining the nascent hydrogen in the material being bleached, nor to any particular temperature, density or thickness, or rate of circulation.

Nor is the invention limited to any specific 55 bisulphites, or acid (other than sulphurous) or reducing material.

The amount of acid, other than sulphurous acid, used, can be varied within wide limits depending on speed of bleaching desired, cost 60 limits, etc. It is advisable, however, to use enough sulphuric acid so that an excess thereof remains when bisulphites of metals whose sulphites are insoluble in neutral or alkaline solution, are used.

65 For example, sulphite pulp cooking acid,

which consists of a mixture of calcium bisulphite, magnesium bisulphite, and free sulphurous acid, can be used as a source of both bisulphites and some of the free sulphurous acid.

To furnish the nascent hydrogen any suitable sources of nascent hydrogen, such as hydrosulphites, zinc, electrolysis, etc., can be used. In this event, the nascent hydrogen is formed in the presence of the pulp.

70 Hydrosulphites, to be added to the pulp, can be conveniently formed from bisulphites, such as sulphite pulp cooking acid or sodium bisulphite, by reduction, by zinc dust or foil, and also by electrolysis.

75 The amount of hydrosulphite used should be small as compared with the amount of bisulphite, in order to prevent the formation of free hydrosulphurous acid, which decomposes into sulphur dioxide and finely divided sulphur, and the presence of the latter may 80 complicate the washing step.

85 The formation of the hydrosulphite may be done either in the bleaching equipment during bleaching or previously, and then 90 added to the mixture.

95 Temperatures between 80 degrees Fahrenheit and 200 degrees Fahrenheit can be used under different conditions; and densities or thicknesses of from 4% bone dry material to 40% bone dry material.

What I claim is:

1. The process of bleaching ground wood pulp, which consists in circulating the pulp in water having mixed therewith a bisulphite, free sulphurous acid, and an acid other than the sulphurous acid, and finally washing the mixture with water until free of acid and other undesired materials.

100 2. The process of bleaching ground wood pulp, which consists in circulating the pulp in water having mixed therewith a bisulphite, free sulphurous acid, an acid other than sulphurous acid, and nascent hydrogen in larger amounts than is given off by the amount of sulphurous acid used, and finally 110 washing the mixture with water until free of acid and other undesired materials.

115 3. The process of bleaching ground wood pulp, which consists in circulating the pulp in water, at densities of from 4% to 40% and at temperatures between 80° F. and 200° F., with a bisulphite, free sulphurous acid, an acid other than sulphurous acid, and nascent hydrogen in larger amounts than is given off by the amount of sulphurous acid used, and then washing the mixture with water until free of acid and other undesired materials.

120 4. The process of bleaching ground wood pulp, which consists in circulating the pulp, at densities of from 4% to 40% and at temperatures between 80° F. and 200° F., in water having mixed therewith a bisulphite, and an acid other than sulphurous 125 acid.

acid, and finally washing the mixture with water until free of acid and other undesired materials.

5. The process of bleaching ground wood pulp, which consists in circulating the pulp in water having mixed therewith sodium bisulphite, concentrated sulphuric acid, and sodium hydrosulphite, and finally washing the mixture until free from acid and other 10 undesired materials.

6. The process of bleaching ground wood pulp, which consists in circulating the pulp in water and in contact with a bleaching agent at densities of from 4% to 40% and 15 at temperatures between 80° F. and 200° F., and then washing the pulp with water until free of acid and other undesired materials.

7. The process of bleaching ground wood pulp, which consists in circulating the pulp in water in contact with a bisulphite, free sulphurous acid, and an acid other than sulphurous acid.

8. The process of bleaching ground wood pulp, which consists in circulating the pulp in water in contact with a bisulphite, free sulphurous acid, an acid other than sulphurous acid, and nascent hydrogen.

9. The process of bleaching ground wood pulp, which consists in circulating the pulp

in water, at densities of from 4% to 40%, in contact with a bisulphite, free sulphurous acid, an acid other than sulphurous acid, and nascent hydrogen.

10. The process of bleaching ground wood 35 pulp, which consists in circulating the pulp in water, at densities of from 4% to 40% and at temperatures between 80° F. and 200° F., in contact with a bisulphite, free sulphurous acid, and an acid other than 40 sulphurous acid.

11. The process of bleaching ground wood pulp, which consists in circulating the pulp in water, at densities of from 4% to 40% and at temperatures between 80° F. and 45 200° F., in contact with a bisulphite, free sulphurous acid, an acid other than sulphurous acid, and nascent hydrogen.

12. The process of bleaching ground wood pulp, which consists in circulating the pulp 50 in water, at densities of from 4% to 40% and at temperatures between 80° F. and 200° F., with a bisulphite, free sulphurous acid, an acid other than sulphurous acid, and finally washing the whole with water 55 until free from acid and other undesired materials.

In testimony whereof I have affixed my signature.

ALFRED O. BRAGG.